

Patented Dec. 2, 1924.

1,517,888

# UNITED STATES PATENT OFFICE.

MAURICE ERNEST BOUVIER, OF LYON, FRANCE, ASSIGNOR TO SOCIETE POUR LA FABRICATION DE LA SOIE RHODIASETA, OF PARIS, FRANCE, A CORPORATION OF FRANCE.

## PROCESS OF TREATING FABRICS FOR REMOVING SIZING OR GUM THEREFROM.

No Drawing.

Application filed July 12, 1923. Serial No. 651,177.

To all whom it may concern:

Be it known that I, MAURICE ERNEST BOUVIER, residing at Lyon, France, a citizen of the Confederation of Switzerland, have invented certain new and useful Improvements in the Processes of Treating Fabrics for Removing Sizing or Gum Therefrom, of which the following is a specification.

10 The threads of artificial silk (cellulose acetate silk and the like) are generally submitted to a treatment intended to render them more adaptable to weaving; by this treatment, they are rendered similar to raw 15 natural silk. This treatment is technically called sizing.

When the threads are woven, it is necessary to remove the sizing therefrom before subjecting them to the preparatory 20 dyeing treatment. Methods for removing the sizing are numerous; for the reason that the sizing methods which are most used, because they are most advantageous for weaving, are not those in 25 which what may be termed the desizing is accomplished in the easiest manner.

In order to desize the fabrics which have been treated for weaving, they must be treated in very hot soap baths, which is 30 very detrimental, as the artificial silk loses its lustre, becomes cotton-like in appearance, and less resistant.

Mixed fabrics of raw natural silk and of 35 artificial silk need also to be thoroughly treated before dyeing or bleaching.

In order to accomplish the degumming of raw natural silk, it is necessary to use a very hot soap bath to which cellulose acetate silk could not be exposed at all; 40 it is therefore necessary, when treating mixed fabrics, to protect the artificial silk against the noxious action of the degumming bath. Moreover, this bath must be absolutely neutral and not contain alkali in 45 any form, or the acetate fibres would be more or less attacked.

It is therefore necessary to avoid adding to the degumming baths sodium carbonate, which salt is often added to accelerate the 50 operation. On the other hand, the agent protecting the artificial silk fibre must not prevent the soap from forming a lather, otherwise its action would be prevented and

the degumming would not take place, or 55 would occur in a very imperfect manner.

Hitherto such an agent was unknown, and it was not possible to dye fabrics of artificial silk, strongly sized, and still less possible to dye mixed fabrics of artificial and raw 60 natural silk. It has been discovered that the addition of neutral salts of potassium (chloride, sulphate, dibasic phosphate, and the like) to the degumming soap bath provides a solution to the problem of protecting 65 the artificial fibre and is satisfactory in every respect.

These salts (in contradistinction to the salts of other metals) have the curious property of not preventing in the least the soap from 70 forming a lather, while they perfectly protect the fibre of cellulose acetate silk, which retains after the treatment all its original properties, even if the temperature of the bath has been raised to 100° C.

75

### Example I.

A fabric of cellulose acetate silk strongly sized is treated in a bath (20 to 60 times the weight of the fabric) containing 0.5 to 2% of neutral soap of the kind known in 80 the trade as "Savon de Marseille" and 5% of potassium chloride. The bath is raised to a temperature of 95-100° C. until the sizing is removed, which requires 30 to 60 85 minutes; the fabric is withdrawn and 901 thoroughly rinsed with soft water.

### Example II.

In Example I, for the potassium chloride is substituted another neutral potassium salt 90 (sulphate, dibasic phosphate or the like).

### Example III.

A mixed fabric of artificial and of raw natural silk is treated in a bath containing 95 0.5 to 2% of neutral soap (Savon de Marseille) and 10% potassium chloride, sulphate or other neutral potassium salt. The temperature is raised to 90-100° C., until the gum of the natural silk and the sizing 98 of the artificial silk are removed and have passed into the bath, which requires from 20 to 60 minutes. The fabric is then withdrawn and rinsed with soft water.

It will be understood that the potassium 98 salts may be used in quantities less than

those mentioned in the examples, and still have a beneficial effect on the preservation of the artificial silk.

If the raw silk contains much gum, one 5 will give a second and lighter soap bath which, replenished, may be used for the first bath in the following operation.

What I claim and desire to secure by Letters Patent is:—

- 10 1. A process of treating fabrics, which consists in subjecting the fabric to a hot soap bath containing a neutral potassium salt.
- 15 2. A process of treating fabrics, which consists in subjecting the fabric to a hot soap bath containing potassium chloride.
- 20 3. A process of treating fabrics, which consists in subjecting the fabric to a hot soap bath containing .5 to 2% of neutral soap and .5 to 10% of potassium chloride.
4. A process of treating fabrics, which

consists in subjecting the fabric to a soap bath containing a neutral potassium salt, and raising the temperature of such bath to 100° C.

25 5. A process of treating fabrics, which consists in subjecting the fabric to a soap bath containing .5 to 2% of neutral soap and from .5 to 10% of potassium chloride, and raising the temperature to 100° C.

30 6. A process for treating mixed fabrics composed of artificial silk fibre and natural raw silk to remove sizing from the former and degum the latter, which consists in subjecting the fabric to a hot soap bath 35 containing a neutral potassium salt.

In testimony whereof I have signed my name to this specification.

MAURICE ERNEST BOUVIER.

Witness:

JULIAN CEMBLE SMEDBERG.